

# UNITED STATES PATENT OFFICE.

FRIEDRICH LUDWIG SCHMIDT, OF CHARLOTTENBURG, GERMANY, ASSIGNOR TO THE  
ROESSLER & HASSSLACHER CHEMICAL COMPANY, A CORPORATION OF NEW YORK.

## PROCESS OF BLEACHING.

1,155,102.

Specification of Letters Patent.

Patented Sept. 28, 1915.

No Drawing. Original application filed January 25, 1910, Serial No. 540,044. Divided and this application filed January 9, 1911. Serial No. 601,695.

To all whom it may concern:

Be it known that I, FRIEDRICH LUDWIG SCHMIDT, a citizen of the German Empire, residing at Charlottenburg, in said German Empire, have invented certain new and useful Improvements in Processes of Bleaching, of which the following is a specification.

This invention relates to an improved process of bleaching by means of borates containing active oxygen in the presence of compounds of magnesium, of the alkaline earth metals and of zinc.

Sodium perborate possesses the property of giving off its oxygen rather rapidly in water at a temperature as low as 50° C. This is a disadvantage in the application of sodium perborate as a bleaching agent, inasmuch as the washing and bleaching process can only properly begin at a higher temperature, so that a large proportion of the oxygen will be driven off and its effect lost before the efficient temperature is attained. In view of this fact, the discovery that magnesium perborate evolves its oxygen at a higher temperature represented an advance.

It is known that mixtures of sodium perborate and a magnesium salt in equivalent proportions can be employed for bleaching, instead of pure magnesium perborate. In this case the magnesium perborate is formed from the sodium perborate and the magnesium salt by double decomposition. The proportions which are used in the latter process are such that the whole of the sodium perborate is decomposed by the magnesium salt. To this extent the latter process only differs from that with magnesium perborate in the fact that the magnesium perborate is produced by the said double decomposition just before the bleaching occurs.

While the employment of magnesium perborate for bleaching purposes represents an advance as regards the bleaching effect, owing to the greater stability of the magnesium perborate under boiling, yet, on the other hand, its high price and some other shortcomings militate against its wide employment.

I have now found that it is possible to obtain the effect of greater resistance to boiling with the cheap sodium perborate and with other alkali metal perborates containing active oxygen, by adding certain substances to the same. To these substances be-

long also the salts of magnesium and their base, magnesia, itself.

The present invention, so far as it extends to the addition of magnesium, differs from the above-mentioned process according to which sodium perborate is completely decomposed by equivalent proportions of magnesium salt.

I have found that it is not necessary to add to the alkali metal perborate so much magnesium compound that the whole bleaching process is carried out with magnesium perborate, that is to say, that all the sodium perborate is decomposed by the magnesium salt. On the contrary, I have found that it is possible to attain the said effect of greater resistance to boiling with only very small proportions of an addition of a magnesium compound. For example, the addition of a fraction of a molecular proportion suffices to attain a very distinct effect, as will appear from the following: A one per cent. solution of sodium perborate, heated to 70-80° C. was found after a few minutes to have lost half of its active oxygen and after twenty-five minutes only 10 per cent. of the oxygen remained. When one-sixth of a molecular proportion of magnesium sulfate is added to one molecular proportion of sodium perborate, dissolved to a one per cent. solution, about 98 per cent. of the active oxygen remains after twenty-five minutes' heating to 70-80°. When under the same conditions one-twelfth of a molecular proportion of magnesium sulfate is added, the effect of this addition is that after twenty-five minutes' heating to the same temperature, about 95 per cent. of the oxygen remains. The addition of one-sixtieth of a molecular proportion of magnesium sulfate under exactly the same conditions has the effect that about 70 per cent. of the oxygen remains after the same period.

It follows from these examples that in order to attain a higher resistance to boiling, it is not necessary to convert the alkali metal perborate completely into magnesium perborate, but, on the contrary, a very small molecular proportion of magnesium salt suffices. This action of less than equivalent proportions of magnesium salt was not to be foreseen, for in the new process, in which the greater portion of the sodium perborate remains unaltered in solution, the natural assumption is that the magnesium salt will decompose the sodium perborate.

tion would therefore be that this unaltered sodium perborate would split off the oxygen just as readily as do ordinary solutions of sodium perborate.

- 5 The new process utilizing only small quantities of magnesium salt is of special importance on account of its technical advantage over the known process using either ready prepared magnesium perborate or  
10 freshly formed magnesium perborate. Both magnesium perborate and the magnesium borate into which the former becomes converted after the bleaching action are insoluble. There is therefore in the bleaching  
15 liquor a considerable quantity of such magnesium precipitate, which, owing to the large quantity present, has a detrimental effect and is difficult to remove from the bleached goods. By using smaller quantities of magnesium salt, far less of this troublesome precipitate has to be dealt with, and the less the quantity of magnesium salt used the smaller is the quantity of the precipitate.  
20  
25 It has further been found that it is not only magnesium alone that possesses the described action, but that compounds of the alkaline earth metals, calcium, strontium, and barium give the same action. This is  
30 illustrated by the following examples carried out under the same conditions as with the sodium perborate, the heating being carried out at the same temperature of 70-80° C. and the remaining oxygen being measured  
35 after twenty-five minutes: The addition of one-sixth of a molecular proportion of chlorid of calcium is found to make the solution stable up to about 87 per cent., while one-fiftieth of a molecular proportion of  
40 chlorid of calcium is found to give a stability of about 50 per cent. One-fifteenth of a molecular proportion of strontium chlorid gives about 90 per cent. stability, one-twelfth of a molecular proportion of barium  
45 chlorid about 80 per cent. stability.
- The following is an example of the bleaching process as carried out by borates containing active oxygen: 200 kilograms of cotton, which is freed in the well-known manner by boiling it with caustic soda from the pectin compounds, is treated with a solution of 2,000 liters of water containing 10 kilos of caustic soda, 5 kilos of soap, 1.5 kilos of sodium perborate, and 0.2 kilo of  
50 crystallized magnesium sulfate, for about five hours in an open vessel, or for from three to four hours under pressure at a temperature of 110° C., under continuous stirring of the mass. After cooling the bleached  
55 cotton is separated from the bleaching liquor, washed and dried.
- 60

In place of the magnesium salt, other salts can be used, as, for instance, 0.3 kilo crystallized calcium chlorid, or 0.27 kilo crystallized strontium chlorid, or 0.25 kilo crystallized barium chlorid. The quantities of these substances can be increased or decreased. In the place of caustic soda, other alkaline substances, as, for instance, soda or Turkey-red oil, can be used. In place of cotton, other vegetable fibers, such as linen, can be treated with advantage by the improved bleaching substances, and also textile fabrics.

The fixing effect of the said substances applies not only to sodium perborate, but also to the other borates containing active oxygen, which can be obtained by crystallization or by mixing or melting. The effect obtained also applies to mixtures of the same with other substances not having a contrary action. The said fixing substances may be added to the active borates and handled or a mixture of both of them, ready for use may be placed upon the market, or the procedure may be such that they are added just before use or during use.

It is not even necessary that the salts or bases having an action in the described sense shall be of the ordinary kind; for example, the persalts and peroxids of the same will serve the purpose.

I wish to be understood that the term "perborate" is also to embrace other borates containing active oxygen, as for instance perborax and such borates, containing active oxygen, as manufactured by the process covered by U. S. Patent No. 1,006,798 issued to me.

Having thus described my invention, I claim as new and desire to secure by Letters Patent:

1. The process herein described of washing and bleaching fibers by means of a perborate, which consists in applying the same to the fibers in the presence of a soluble inorganic compound of magnesium in a less than equivalent proportion.

2. The process herein described of washing and bleaching fibers by means of a perborate, which consists in applying the same to the fibers in the presence of a soluble inorganic compound of an alkali earth metal in a less than equivalent proportion.

In testimony, that I claim the foregoing as my invention, I have signed my name in presence of two subscribing witnesses.

FRIEDRICH LUDWIG SCHMIDT.

Witnesses:

REINHOLD GRUBER,  
MAX MAETSCHKE.